

Dec. 15, 1942.

W. S. MARX, JR

2,304,838

PHOTOENGRAVING

Filed Jan. 4, 1940

Fig. 1.



Fig. 2.



Fig. 3.



INVENTOR.  
Walter S. Marx Jr.  
BY Parkinson + Lane  
ATTORNEY.

## UNITED STATES PATENT OFFICE

2,304,838

## PHOTOENGRAVING

Walter S. Marx, Jr., Park Ridge, Ill., assignor to  
Printing Arts Research Laboratories, Inc., Chi-  
cago, Ill., a corporation of Delaware

Application January 4, 1940, Serial No. 312,343

8 Claims. (Cl. 95—5)

This invention relates to photo-engraving, and more particularly to a method of forming highlight negatives for half-tone printing plates as well as to means for preparing drawings from which such negatives can be produced. This application is a continuation in part of my application Serial No. 209,492, which resulted in Patent No. 2,191,939.

An object of this invention is to provide a simple method of "highlighting" that is free from the more lengthy and inexpedient prevailing methods, such as laborious hand-painting or hand-opaquing, or which involve the employment of special lenses and stops that are in many instances impractical and depend upon delicately balanced exposure relationships, and which in any event are limited to the reproduction of certain types of copy only.

A further object of the invention is to provide a method of, and means for, greatly reducing the cost of highlight half-tone printing plates by decreasing the production time, and substituting for the present difficult manual method of highlighting, an efficient photo-automatic procedure.

Briefly, the method of this invention consists in the removal of half-tone pattern in the highlight areas by means of a double exposure of the light-sensitive element or negative in a camera, the first of said exposures being through a half-tone screen in the usual way, whereby all tones of the subject in proper values are correctly recorded, and the second exposure with the half-tone screen effectually removed and by means of light changed in frequency by a molecular change in energy levels resulting from the inclusion of predetermined substances in the work areas of the drawing or subject to be photographed, as will hereinafter be disclosed in detail, the non-work or highlight areas remaining unchanged and are thus photographed in said second exposure to the extent required to effectually cover or efface the latent half-tone record or "highlight" dots of the first exposure without affecting the half-tone pattern in the work areas.

The first of the above mentioned exposures is made in the presence of visible or ordinary light whilst the second exposure is made in the presence of light rays lying outside of the visible spectrum, that is to say, rays outside the visible spectrum at its violet end, namely, ultra-violet rays, or those rays which lie just beyond said spectrum at its red end, namely, infra-red rays.

The order of the two exposures may, of course, be reversed, as will be understood.

A further object of this invention is to improve the accuracy of reproduction of highlight drawings and similar illustrative matter by the employment of a marking device, such as a pencil.

To this end the present invention also relates to a pencil, the marking material of which in-

cludes a substance which will absorb infra-red light or ultra-violet light in such a way that when the markings made by the pencil are photographed by means of such light and with visible or white light in the manner already outlined in connection with the method of this invention above, a highlight half-tone printing plate may be made photo-automatically from a drawing or subject prepared with such pencil.

The word "pencil" is used herein for convenience of description and is therefore to be considered as including in meaning all types of marking devices, such as crayons, pastels, pencil "leads," pens, quills, etc., the markings of which may be applied in either liquid or solid phases, or both.

A "highlight half-tone printing plate" as herein used is to be understood to mean, as it does in the art, a screened printing plate which is free of dot pattern or other half-tone scanning in the background and/or highlighted areas of the matter so reproduced.

Furthermore, it is to be considered for the purpose of description herein that ultra-violet and infra-red energy forms are actually light waves, and that as such they may be measured, used, and theoretically calculated for conclusions demonstrable from that basis.

Other objects and advantages of the invention will be apparent from the following detailed description, by referring to the accompanying drawing, in which:

Figure 1 is an enlarged section of a marking made with the pencil of this invention, and

Figures 2 and 3 are structural formulae showing the chemical constitution of markings made with a pencil of this invention, Figure 2 representing para-hydroxybenzaldehyde, and Figure 3 representing anthracene, each compound being typical in general of intra-molecular and inter-molecular energy absorption materials respectively, and each figure shows the behavior of these materials during the herein described work thereon, and under the influence of light energy.

According to this invention, the following formula may be used for making up a pencil, the markings of which, when made alkaline, will effectually absorb ultra-violet light:

|                                                                            | Parts by weight |
|----------------------------------------------------------------------------|-----------------|
| Kaolin                                                                     | 30              |
| Graphite                                                                   | 8               |
| Carbon black (or other pigment)                                            | 18              |
| Beta-methyl-umbelliferone                                                  | 40              |
| Phenanthrene                                                               | 23              |
| Sodium stearate                                                            | 16              |
| Anime (Indian gum)                                                         | 5               |
| Extrude under heavy pressure at 170 to 180 degrees C. Dry for fifty hours. |                 |
| After the drawing to be reproduced has been                                |                 |

prepared with a pencil as above made up it is sprayed or otherwise coated with an alkalinizing material. A preferred method is to spray the drawing with a volatile alkalinizing compound, made as follows:

| Parts by volume           |    |
|---------------------------|----|
| Isopropyl alcohol         | 85 |
| Chemically pure glycerine | 10 |
| Morpholine                | 5  |

This spraying compound is preferred because the alkaline material volatilizes off, leaving the markings made by the pencil and supporting surface thereof in a more neutral and consequently more stable condition, since most drawing papers oxidize more rapidly in an alkaline state.

Each microscopic particle, or group of particles, in the marking made by the pencil indicated, for example, at A in Figure 1, contains beta-methyl-umbelliferone. This material, being very soluble in bases and alcohols, is dissolved out by the alkaline-alcohol spray which is applied over the marking. The detergent nature of this resulting solution tends to spread the solutes beyond the normal periphery of the original particle A. Thus, on a surface supporting the marking, the region bounded on its outer limits by the farthest spread of the above solution indicated by B, and on its inner limits by the periphery of the particle A is effectually transparent to white light, and effectually absorbent of ultra-violet light.

Thus, if A in Figure 1 is black (as in the case of a black pencil) it will absorb both white and ultra-violet light; whereas region B as defined above will absorb only in the ultra-violet. Therefore, if region B is five times the area of region A, the region AB will absorb six times more ultra-violet light than white light.

The theory upon which the present invention is based hinges upon just that amplification of light absorption. The relative numerical value of absorption quanta is, of course, dependent directly upon the area ratio of B to A. Also, the spread of the umbelliferone solution over B, and determining the size of B, is controlled by the nature and quantity of the alkalinizing spray.

The manner in which the above light absorption principle can be utilized as a means for photo-automatic production of highlight half-tone printing plates is as follows:

The drawing or marking of which region AB is a part, is photographed in two steps, the first step comprising the normal series of half-tone exposures through proper lens diaphragms and half-tone screen, and using white light in the normal manner, thus recording upon the negative element a half-tone record of the marking or drawing made with the present pencil; The second step being an auxiliary exposure superimposed upon the record of the first step, and made by means of ultra-violet light only and with the half-tone screen effectually removed from the system. The ultra-violet light reflected from all regions around AB will record continuously over all corresponding regions on the negative element, thus "veiling over" or covering up the heretofore unexposed "openings" on the negative element which were projected thereon by the half-tone screen in the first step. The screen pattern, or dots, are thereby effectually eliminated in all areas on the negative element corresponding to the unmarked or effectually untreated areas on the surface supporting the marking.

Conversely, the region AB will have little or no appreciable effect on the negative element during the exposure by ultra-violet light only, since this area does not effectually reflect ultra-violet light, but rather absorbs it, due to energy transference which may be explained as follows:

It may be contended that all light absorption is the result of inter or intra molecular energy absorption, directly or indirectly. This is more especially true of the energy transference involved for the purpose of this invention. Therefore, the application of both types of energy absorption will be explained, and the use of any materials absorbing light in such manner, when used for the same purpose and to the same end as that herein disclosed, is considered as within the scope of this invention.

In Figure 1, region B is covered with the umbelliferone solution as previously described. The residual salt of this umbelliferone solution may be represented structurally by either an ortho or para quinonoid formula. Since the structural formula for beta-methyl-umbelliferone is, in this connection, highly complex, the equivalent and simpler formula will be given with reference to Figure 2 for para hydroxybenzaldehyde as an example of intra molecular energy absorption.

Figure 2 shows para hydroxybenzaldehyde in a neutral condition and its configuration in an alkaline condition, and the consequent change to a quinonoid structure. The phenolic hydrogen is ionized off, leaving the negative ion, which can exist in the two forms shown by shifting from one oxygen atom to another. It is that mobile electron and the quinonoid structure resulting from its movement which absorbs light. Or when the phenolic oxygen holds the electron, as in state I, the energy is presumably lower than when the electron is on the aldehydic oxygen, and incident light provides sufficient energy to bring state I to state II.

In general this electronic activity is indicative of the action of many light-absorbing compounds of the intra-molecular energy absorption type, where the free electron or electrons go from one or more energy levels to another, such as quinine sulfate, fluorescein, copper sulfate, and nearly all rare earth salts, etc.

Figure 3 illustrates an example of intermolecular energy absorption, in this case anthracene, and shows the behavior of such compounds of the same absorption group as, for instance, phenanthrene, ortho nitrobenzaldehyde, cinnamidine carboxylic acid, etc. The mono-molecular forms of these compounds absorb energy to carry them over to the di-molecular forms, and, as described herein, photographic use is made of that energy absorption.

Some further energy absorbing compounds which may be used to the same end, and which absorb in situ, such as the potassium salt of para hydroxybenzaldehyde in the intra molecular group, or such as anthracene in the inter molecular group, are optional embodiments of this invention, because these compounds are, per se, in an energy absorbing state. Also, compounds which absorb energy through decomposition are considered within the scope of this invention, as falling within the above circumscribed limits of molecular energy absorption characteristics. In brief, any light absorbing or energy absorbing material or materials, when used to achieve the herein described end, irrespective of the procedure employed, are considered as falling within the scope of the present invention.

A marking device according to the present invention, the inscription of which is absorbent of infra-red radiations, may be made as follows:

|                | Grams |
|----------------|-------|
| Kaolin         | 27    |
| Benzoic acid   | 30    |
| Phenanthrene   | 15    |
| Copper sulfate | 20    |
| Gum anime      | 5     |
| Graphite       | 5     |
| Pigment        | 10    |

and five grams of the following:

|               | Parts |
|---------------|-------|
| White beeswax | 3     |
| Carnauba wax  | 5     |

This mixture is heated to 180° C. and extruded at high pressure and dried in any manner well known in the art for 50 hours.

Variations of the above formula including infra-red absorbents other than copper sulfate, may be used to the same end.

Moreover, sprays or coatings of materials intended to spread such infra-red absorbent beyond its otherwise normal confiner—(as has been shown in the case of the ultra-violet absorbents)—are also required in this case. To spread copper sulfate particles for instance, water and alcohol may be used in equal parts. The spray or coating will, of course, in any case contain an effective quantity of a solvent in which the absorbent used is very highly soluble, and also a detergent capable of spreading the solution so formed, beyond its otherwise normal periphery.

It will be understood that any suitable infrared sensitizing dye is included in the photo-sensitive element used for the photography of inscriptions made by the above marking device aforescribed and, furthermore, that infra-red light will be substituted for the ultra-violet light utilized as hereinbefore described in connection with the employment of a marking device containing an absorbent of the latter light.

I claim:

1. Method of half-tone photography which comprises the steps of making a drawing from which a half-tone printing plate is to be prepared with a marking device, the marking material of which includes a pigment and a substance capable of absorbing light lying outside of the visible spectrum, treating the drawing with a material adapted to render said substance more effective to absorb said light, photographing the drawing so prepared and treated on a light-sensitive element in accordance with the usual half-tone procedure and then superimposing on said light-sensitive element a second image of said drawing in the presence of light rays lying outside of the visible spectrum corresponding to those which the drawing has been rendered effective to absorb.

2. Method of half-tone photography which comprises the steps of making a drawing from which a half-tone printing plate is to be prepared with a marking device, the marking material of which includes a pigment and a substance capable of absorbing light lying outside of the visible spectrum, treating the drawing with a solution adapted to render said substance more effective to absorb said light and capable of amplifying the area of the drawing over which said absorbent action is effective, photographing the drawing so prepared and treated on a light-sensitive element in accordance with the usual half-tone procedure and then superimposing

on said light-sensitive element a second image of said drawing in the presence of light rays lying outside of the visible spectrum corresponding to those which the drawing has been rendered effective to absorb.

3. Method of half-tone photography which comprises the steps of making a drawing from which a half-tone printing plate is to be prepared with a marking device, the marking material of which includes a pigment and a substance capable of absorbing ultra-violet light, treating the drawing with a material adapted to render said substance more effective to absorb said light, photographing the drawing so prepared and treated on a light-sensitive element in accordance with the usual half-tone procedure and then superimposing on said light-sensitive element a second image of said drawing in the presence only of ultra-violet light.

20 4. Method of half-tone photography which comprises the steps of making a drawing from which a half-tone printing plate is to be prepared with a marking device, the marking material of which includes a pigment and a substance capable of absorbing infra-red light, treating the drawing with a material adapted to cause said substance to diffuse, photographing the drawing so prepared and treated on a light-sensitive element in accordance with the usual half-tone procedure and then superimposing on said light-sensitive element a second image of said drawing in the presence only of infra-red light.

30 5. Method of half-tone photography which comprises the steps of making the drawing from which a half-tone printing plate is to be prepared with a marking device, the marking material of which includes a pigment and beta-methyl-umbelliferone, applying an alkalizing material to the drawing so prepared, photographing said drawing on a light-sensitive element in accordance with the usual half-tone procedure and then superimposing on said light-sensitive element a second image of said drawing in the presence only of ultra-violet light.

45 6. A method of half-tone photography for eliminating screen pattern in the highlight portions of a half-tone negative, comprising incorporating in a marking device a pigment and an absorbent of light rays lying outside of the visible spectrum, preparing a drawing to be photographed with the aid of said marking device, photographing said drawing on a light-sensitive element in accordance with the usual half-tone procedure, and then superposing on said element and in register with the first image, a second image of said drawing in the presence only of light rays lying outside of the visible spectrum corresponding to those which the drawing has been rendered effective to absorb.

50 7. Method of half-tone photography for eliminating screen pattern in the highlight portions of a half-tone negative, comprising incorporating in a solid marking device a pigment and an absorbent of light rays lying outside of the visible spectrum, preparing a drawing to be photographed with the aid of said marking device, thereby producing on the drawing shaded portions constituted by a plurality of discrete separate particles of the marking device, treating the drawing with a solvent for said substance whereby some of said substance included within said discrete particles is dissolved and distributed over areas of the drawing around and adjacent said discrete particles, photographing said drawing on a light sensitive element with two sepa-

rate registering exposures, one of said exposures being effected with the aid of a screen in accordance with usual half-tone procedure, the other of said exposures being made with the screen effectually removed and with the air only of light rays lying outside of the visible spectrum and corresponding to those which the drawing has been rendered effective to absorb, the last-mentioned exposure being made after the solvent treatment of the drawing.

8. Method of half-tone photography for eliminating screen pattern in the highlight portions of a half-tone negative, comprising incorporating in a solid marking device a pigment and an absorbent of ultra-violet light rays, preparing a drawing to be photographed with the aid of said marking device, thereby producing on the draw-

ing shaded portions constituted by a plurality of discrete separate particles of the marking device, treating the drawing with a solvent for said substance whereby some of said substance included within said discrete particles is dissolved and distributed over areas of the drawing around and adjacent said discrete particles, photographing said drawing on a light-sensitive element with two separate registering exposures, one of said exposures being effected with the aid of a screen in accordance with usual half-tone procedure, the other of said exposures being made with the screen effectually removed and with the aid of ultra-violet light only, the last-mentioned exposure being made after the solvent treatment of the drawing.

WALTER S. MARX, Jr.